

## UNITED STATES PATENT OFFICE

2,687,350

TITANIUM BASE ALLOYS CONTAINING  
CHROMIUM AND CARBON

Charles M. Craighead, Columbus, Ohio, assignor,  
by mesne assignments, to The Battelle Development  
Corporation, Columbus, Ohio, a corporation  
of Delaware

No Drawing. Application October 6, 1950,  
Serial No. 188,891

2 Claims. (Cl. 75—177)

**1**  
This invention relates to titanium-base alloys and, more particularly, to titanium-base alloys containing chromium and carbon, and is a continuation-in-part of co-pending application, Serial No. 36,434, filed July 1, 1948, now abandoned. 5

It has become generally recognized that titanium metal possesses valuable properties which render it desirable for various structural uses and for other purposes. For example, the metal has an excellent strength/weight ratio, good corrosion properties, and is useful for high-temperature applications. However, these various properties of titanium are not ordinarily subject to adjustment to meet specific requirements imposed by particular applications. For this reason then, 15 as well as for purposes of improving the properties of the base metal, it is desirable to produce alloys of titanium which will possess desired properties in the required degree, or which will respond to heat treatment, or other methods for enhancing a particular quality (characteristic) or property.

It is accordingly an object of this invention to provide alloys of titanium containing chromium and carbon.

It is another object of this invention to provide titanium-chromium-carbon alloys having desirable properties for structural or other purposes.

Yet another object of this invention is to produce titanium-chromium-carbon alloys which are responsive to heat treatment.

Other objects and advantages of the present invention will be apparent in view of the following detailed description thereof.

In general, this invention relates to alloys of titanium containing chromium and carbon. In particular, the invention relates to titanium alloys containing from about 1.5% to about 7.5% chromium and from about 0.2% to about 0.6% carbon. A preferred range of from 2.5% to 5.0% chromium and 0.25% to 0.5% carbon has also been established.

Titanium-chromium-carbon alloys may be prepared in accordance with present-day melting techniques which form no part of the present invention and need not be discussed further here.

Table I below lists typical values obtained in physical tests of titanium-chromium-carbon al-

loys. Properties listed are the as-hot-rolled values (at 1450° F.).

Table I

| Composition <sup>1</sup> |           |                     |           | Tensile Strength, p. s. i. | Elongation, percent in 1-in. | V. H. N. |  |  |  |
|--------------------------|-----------|---------------------|-----------|----------------------------|------------------------------|----------|--|--|--|
| Intended                 |           | Actual <sup>2</sup> |           |                            |                              |          |  |  |  |
| Percent Cr.              | Percent C | Percent Cr          | Percent C |                            |                              |          |  |  |  |
| 2.5                      | 0.25      | 2.25                | 141,400   | 7.5                        | 305                          |          |  |  |  |
| 2.5                      | 0.25      | 2.28                | 171,200   | 8.0                        | 336                          |          |  |  |  |
| 3.5                      | 0.25      | 3.23                | 160,200   | 5.0                        | 262                          |          |  |  |  |
| 5.0                      | 0.25      | 4.94                | 179,900   | 5.0                        | 349                          |          |  |  |  |
| 5.0                      | 0.25      | 4.27                | 158,100   | 6.5                        | 288                          |          |  |  |  |
| 10.0                     | 0.25      | 9.40                | 179,400   | 3.5                        | 383                          |          |  |  |  |
| 15.0                     | 0.25      | 14.40               | 171,000   | 6.0                        | 346                          |          |  |  |  |
| 2.5                      | 0.50      | 2.15                | 128,200   | 11.5                       | 245                          |          |  |  |  |
| 3.5                      | 0.50      | 3.35                | 146,900   | 7.0                        | 266                          |          |  |  |  |
| 5.0                      | 0.50      | 4.21                | 155,300   | 5.0                        | 280                          |          |  |  |  |

<sup>1</sup> Balance Ti.<sup>2</sup> No analysis made for C.

From the table above, it will be apparent that titanium-chromium-carbon alloys in the preferred range possess good tensile properties combined with sufficient ductility to permit ordinary working of the alloys. Furthermore, alloys in the range 1.5% to 7.5% chromium, 0.2% to 0.6% carbon, the balance essentially all titanium, possess these properties, although to a slightly lesser degree. These alloys also have the corrosion resistance and other desirable properties ordinarily imputed to titanium and titanium alloys.

That the alloys of the present invention respond to heat treatment is indicated by the data in Table II, wherein it will be noted that the hardness is generally increased by heat treatment at temperatures in the range 1450° F. to 1750° F., and also by aging at 750° F. for various periods of time ranging from two to twelve hours. The particular heat treatment which effected the hardness changes reported consisted of heating specimens in air for 30 minutes at the designated temperature and then quenching in cold water. Each value reported represents the average of at least five readings taken at the center of a cross-section perpendicular to the direction of rolling.

Table II

| Composition   |              |               |              | V. H. N.<br>as Hot-<br>Rolled | Anneal,<br>1,450° F. | Vicker's Hardness Number After Heat<br>Treatment <sup>1</sup> At— |           |           |           |           | V. H. N. as Hot-Rolled and Aged<br>at 750° F. for— |         |         |         |         |          |
|---------------|--------------|---------------|--------------|-------------------------------|----------------------|-------------------------------------------------------------------|-----------|-----------|-----------|-----------|----------------------------------------------------|---------|---------|---------|---------|----------|
| Intended      |              | Actual        |              |                               |                      | 1,450° F.                                                         | 1,550° F. | 1,600° F. | 1,650° F. | 1,700° F. | 1,750° F.                                          | 0 Hours | 2 Hours | 4 Hours | 8 Hours | 12 Hours |
| Percent<br>Cr | Percent<br>C | Percent<br>Cr | Percent<br>C |                               |                      |                                                                   |           |           |           |           |                                                    |         |         |         |         |          |
| 2.5           | 0.25         | 2.25          | 0.28         | 305                           | 304                  | 301                                                               | 318       | 314       | 327       | 339       | 369                                                | 305     | 318     | 363     | 385     | 327      |
| 2.5           | 0.25         | 2.28          | 0.28         | 336                           | 304                  | 307                                                               | 352       | 320       | 321       | 319       | 377                                                | 326     | 354     | 363     | 385     | 327      |
| 3.5           | 0.25         | 3.23          | —            | 262                           | —                    | 312                                                               | 352       | 320       | 321       | 319       | 380                                                | 262     | 345     | 345     | 352     | —        |
| 5.0           | 0.25         | 4.94          | 0.25         | 349                           | 353                  | 386                                                               | —         | —         | —         | —         | 392                                                | 353     | 383     | 387     | 398     | 352      |
| 5.0           | 0.25         | 4.27          | —            | 288                           | —                    | 310                                                               | 376       | 303       | 309       | 312       | 314                                                | 288     | 357     | 357     | —       | —        |
| 10.0          | 0.25         | 9.40          | 0.28         | 383                           | 443                  | 326                                                               | —         | —         | —         | —         | 333                                                | 376     | 506     | 503     | 482     | 456      |
| 15.0          | 0.25         | 14.40         | 0.13         | 346                           | 337                  | 334                                                               | —         | —         | —         | —         | 370                                                | 317     | 465     | 459     | 488     | 427      |
| 2.5           | 0.5          | 2.15          | —            | 245                           | —                    | 257                                                               | 291       | 294       | 297       | 306       | 302                                                | 245     | —       | 301     | —       | —        |
| 3.5           | 0.5          | 3.35          | —            | 286                           | —                    | 296                                                               | 295       | 277       | 311       | 313       | 335                                                | 266     | —       | 321     | —       | —        |
| 5.0           | 0.5          | 4.21          | —            | 280                           | —                    | 355                                                               | 305       | 301       | 362       | 446       | 366                                                | 280     | —       | 355     | —       | —        |

<sup>1</sup> Balance titanium.<sup>2</sup> Held at indicated temperature for 30 minutes and quenched in cold water.

It will now be apparent that new and useful 20 alloys of titanium, chromium, and carbon have been described wherefore it will be obvious to those skilled in the art that certain slight changes may be made without departing from the scope 25 of this invention which is hereinafter defined in the claims.

What is claimed is:

1. An alloy consisting essentially of from about 1.5% to about 7.5% chromium, from about 0.2% to about 0.6% carbon, and the balance titanium, 30 said alloy being characterized by having a minimum tensile strength of about 128,200 p. s. i. and a minimum elongation of about 5.0% in the as-hot-rolled (at 1450° F.) condition.

2. An alloy consisting of from about 2.5% to about 5.0% chromium, from about 0.25% to about 0.50% carbon, and the balance titanium.

#### References Cited in the file of this patent

#### UNITED STATES PATENTS

Number Name Date  
1,471,326 Copland ----- Oct. 23, 1923

#### OTHER REFERENCES

Zeitschrift fur Metallkunde, vol. 29 (1937), page 190.

"Metal Progress," March 1949, page 348.

"Metal Progress," November 1949, page 658.

"Product Engineering," November 1949, page 148.

"Industrial and Engineering Chemistry," February 1950, pages 222-226, 243.

**Notice of Adverse Decision in Interference**

In Interference No. 87,804 involving Patent No. 2,687,350, C. M. Craighead, Titanium base alloys containing chromium and carbon, final judgment adverse to the patentee was rendered April 9, 1957, as to claim 1.

*[Official Gazette May 21, 1957.]*